# EUROPEAN PATENT SPECIFICATION

(11) **EP 3 112 486 B1**
(45) Date of publication and mention of the grant of the patent: **05.06.2019**
(21) Application number: 15743006.7
(22) Date of filing: 28.01.2015
(51) Int. Cl.: C22C 32/00, C22C 21/00, C22C 1/10, B21B 1/46

(54) **METHOD OF PRODUCING B 4C/AL NEUTRON ABSORBENT MATERIAL SHEET BY CONTINUOUS CAST ROLLING**
VERFAHREN ZUR HERSTELLUNG EINER B-4C/AL-NEUTRONENABSORBIERENDEN MATERIALBAHN DURCH STRANGGIESSWALZEN
PROCÉDÉ DE PRODUCTION D'UNE FEUILLE DE MATÉRIAU ABSORBANT NEUTRONIQUE B 4C/AL PAR LAMINAGE EN COULÉE CONTINUE

(30) Priority: 28.01.2014 CN 201410042799
(43) Date of publication of application: 04.01.2017
(73) Proprietor: China Nuclear Power Engineering Company Ltd., Shenzen, Gaungdong 518023 (CN); Graduate School at Shenzhen, Tsinghua University, Shenzhen, Guangdong 518055 (CN); China General Nuclear Power Corporation, Shenzhen, Guangdong 518031 (CN)
(72) Inventor: SHU, Guogang, Shenzhen Guangdong 518023 (CN); LI, Qiulin, Shenzhen Guangdong 518055 (CN); LUO, Zhiyuan, Shenzhen Guangdong 518023 (CN); LIU, Wei, Shenzhen Guangdong 518055 (CN); LIU, Yanzhang, Shenzhen Guangdong 518023 (CN); WANG, Xin, Shenzhen Guangdong 518023 (CN); LI, Xuejun, Shenzhen Guangdong 518023 (CN); ZHANG, Tengfei, Shenzhen Guangdong 518055 (CN)
(74) Representative: Greaves Brewster LLP
(86) International application number: PCT/CN2015/071767
(87) International publication number: WO 2015/113502

(56) References cited:
- EP-A1- 0 437 153
- WO-A2-2004/038050
- CN-A- 1 140 766
- CN-A- 1 708 597
- CN-A- 103 273 026
- CN-A- 103 789 599
- JP-A- 2012 096 289
- US-A1- 2011 247 778
- US-A1- 2012 121 890
- US-B1- 6 253 831
- N V Murthy ET AL: "A REVIEW ON FABRICATION OF ALUMINIUM ALLOY BASED METAL MATRIX NANO COMPOSITES THROUGH ULTRASONIC ASSISTED CASTING", , 1 December 2012 (2012-12-01), XP055412691, Retrieved from the Internet: URL:http://www.tjprc.org/publishpapers/--1 469098741-1. JMMR - A Review on Fabrication of Aluminium alloy based Metal Matrix.pdf [retrieved on 2017-10-05]
- WANG, LAOHU: 'Study on Preparation, Microstructures, and Properties of Magnesium Matrix Composites under Physical External Fields' MASTER'S DISSERTATION OF DALIAN UNIVERSITY OF TECHNOLOGY 30 September 2013, pages 13 - 15, XP008184593

## Description

### TECHNICAL FIELD

The present invention generally relates to composites and, more particularly, to a method for producing B4C/A1 neutron-absorbing material sheet by continuous cast rolling.

### BACKGROUND

In nuclear energy technical field, nuclear fuel in the reactor will turn into spent fuel after a certain amount of working time. The unloaded spent fuel having very strong radiation needs to be stored properly. Sheet of B4C/A1 composite having high content of B4C has been widely used in commercial application as neutron-absorbing material for storing spent fuel. The performances of B4C/A1 composite mainly depends on the mass content of B4C particles, the dispersion of the B4C particles in the matrix, the interface of the matrix and the B4C particles, as well as the microstructure of the matrix.

At present, methods for producing B4C/A1 neutron-absorbing material mainly includes powder metallurgy method, melt infiltration method and stirring casting method, in which stirring casting method is the most promising method for producing B4C/A1 neutron-absorbing material due to high production efficiency, simple process flow and suitability for mass production.

Conventional stirring casting method for producing B4C/A1 composite generally includes the steps of aluminum ingot smelting, mixing the composite, casting, saw cutting and surface milling, heating, cogging and hot rolling. Generally, the production efficiency and degree of automation of the conventional stirring casting method for producing B4C/A1 composite are very low. Due to the slow cooling rate in the casting process, uniformity of the B4C particles in the B4C/A1 composite sheet is unsatisfactory, which may adversely affect neutron absorbing property and other mechanical properties of the B4C/A1 composite.

In mass production, the solidification rate of alloy in conventional casting billet producing method is very slow, which will inevitably lead to some defects, such as microstructure segregation. The aluminum matrix melt containing high mass content of B4C particles has large viscosity and poor fluidity. During the casting process, the aluminum matrix melt containing high mass content of B4C particles can't feeding in time, which may lead to defects, such as contraction cavities and shrinkage porosity. In addition, the B4C particles acting as heterogeneous cores have poor wettability in the aluminum matrix. During the solidification process, due to the crowding out effect of the matrix solidification front to the B4C particles, the B4C particles cannot disperse uniformly in the aluminum matrix.

Twin roll continuous cast rolling is a molding process which has the advantages of the rapid solidification and hot rolling deformation. During twin roll continuous cast rolling, the cast rolls act as crystallizer and hot rolls. In casting rolling, the solidification rate of the liquid metal is very high (as high as103-104°C/s), so that the reinforcement can distribute homogeneously in the matrix and the defects in the composite are reduced remarkably, which not only can improve the strength of the composite, but also can ensure the ductility and deformability of the material.

X. Grant Chen et al. of Alcan Company (company of Canada) disclose in "DEVELOPMENT OF Al-30% B4C METAL MATRIX COMPOSITES FOR NEUTRON ABSORBER MATERIAL" that sheet of B4C/A1 composite having 30% B4C by mass can be produced via stir-mixing process in laboratory and extrusion or hot rolling process. However, during solidification, the B4C particles intend to gather in the center area. Even extrusion or hot rolling process can improve uniformity of the B4C particles, the B4C/A1 composite, especially B4C/A1 composite having high mass content of B4C particles, has high hardness and poor deformation processing performances and, therefore, it is difficult to produce sheet via cold rolling. At present, repeated hot rolling is implemented on casting ingots, which will remarkably increase the producing cost.

NIE cun zhu of Shanghai Jiao Tong University discloses a method for producing a B4C/Al composite containing 10% by volume of B4C particles via stirring method in his Ph. D. theses, titled "Research of Fabrication and Weldability of Boron Carbide Particulates Reinforced Aluminum Matrix composites". However, due to severe interface reaction, the mechanical properties of the composite are poor and the volume content of the B4C particles is not high enough. Japanese scholar T. Haga discloses in an article titled "Roll casting of Al-SiCp strip" that after stirring and mixing, twin roll continuous cast rolling technology is used to directly roll the composite containing 20% and 30% by volume of SiCp, so as to obtain a sheet material having a thickness of 2.0mm and 1.7mm. The uniformity of the particles in the sheet material is higher than that of the sheet material produced by conventional casting methods. In addition, the sheet material is suitable for following cold rolling or hot rolling. However, analysis shows that the uniformity of the particles in the sheet material after continuous rolling is still not satisfactory enough.

US2011/247778 discloses a method of synthesizing particle reinforced metal matrix composite material by in-situ melt reaction in coupling magnetic field and ultrasonic field. The method comprises adjusting metal-base melt to the onset reaction temperature after refining, then adding reactants which generate reinforced particles by in-situ synthesis reaction with melt, keeping the reacted melt stand until it is cooled to casting after the reaction, and then casting. Magnetic field and high-energy ultrasonic field are exerted simultaneously during the reaction.

US6253831 discloses a casting process for producing a metal matrix composite having a first phase matrix of metal or metal alloy containing second phase particles dispersed therein. The method comprises the steps of preparing a melt of the metal or metal alloy in the vessel, feeding the particles to the melt; applying ultrasonic vibration to the melt while electromagnetically stirring the melt and then causing solidification of the melt.

In view of the foregoing, what is needed, therefore, is to provide a method for producing B4C/Al neutron-absorbing material sheet by continuous cast rolling which can ensure uniform distribution of B4C particles in the aluminum matrix.

### BRIEF SUMMARY OF VARIOUS EMBODIMENTS OF THE INVENTION

One object of the present invention is to provide a method for producing B4C/A1 neutron-absorbing material sheet by continuous cast rolling which can ensure uniform distribution of B4C particles in the aluminum matrix.

According to one embodiment of the present invention, a method for producing B4C/AL neutron -absorbing material sheet by continuous cast rolling including the steps of:
1) providing B4C particles and aluminum matrix melt, adding the B4C particles into the aluminum matrix melt while stirring the composite of the B4C particles and the aluminum matrix melt;
2) applying an electromagnetic field to the B4C particle-containing aluminum matrix melt passing through a headbox to achieve electromagnetic dispersion;
3) applying an ultrasonic vibration to the B4C particle-containing aluminum matrix melt passing through a casting nozzle; and
4) conducing twin roll continuous cast rolling on the B4C particle-containing aluminum matrix melt from the casting nozzle to obtain a B4C/A1 neutron-absorbing material sheet, and
wherein a mass content of the B4C particles in the B4C/A1 neutron-absorbing material sheet is 20-31%.

Via applying ultrasonic vibration during cast rolling process, due to the acoustic cavitation and the acoustic streaming effect, air bubbles in the aluminum matrix melt can be reduced remarkably, which can spheroidize and refine the solidified grains. The energy applied by the ultrasonic to the interface of the aluminum matrix melt and the B4C particles can promote wettability of the aluminum matrix melt on the B4C particles. Local high temperature and high pressure caused by the acoustic cavitation can clean and activate the surface of the B4C particles, so as to increase the surface energy of the particles and reduce the surface energy of the melt. The stirring of the acoustic streaming realizes macro uniform dispersion of the B4C particles. The comprehensive effect of the acoustic cavitation and the acoustic streaming can realize micro uniform dispersion of the B4C particles.

The headbox of the continuous cast rolling equipment is positioned in the space between the upper and lower iron cores. When direct current passes through the aluminum liquid and alternating current passes through the coils, the electromagnetic induction device will generate an alternating traveling magnetic field along the axis direction of the rolls and a vertical oscillating magnetic field, mainly the traveling magnetic field. In non-contact condition, the aluminum liquid generates induced current due to the changing magnetic field, which will lead to generation of changing electromagnetic force and movement of the particles in the aluminum matrix liquid. According to electromagnetism principle, complex magnetic field mainly including the traveling magnetic field and the electromagnetic induction applied to the cast rolling zone will generates horizontal stirring force parallel to the axis direction of the rolls. Via changing the direction of the traveling magnetic field, the direction of the stirring force can be changed, which will lead to abnormal and small amplitude migration flow in the solidification zone of the solidification front, so that the flow field, the temperature field and the concentration field of the melt change constantly. The changing flow field, temperature field and concentration field of the melt will provide scouring force and mechanical shear force to the dendritic at the solidification front, and leads to peel off and break of the dendritic and increases nucleation centers. Therefore, applying electromagnetic field during the continuous casting process can obtain composite sheet having refined and equiaxed grains and uniformly dispersed B4C particles.

According to one aspect of the present invention, a particle size of the B4C particles is 0-44µm.

According to one aspect of the present invention, in step 1), the aluminum matrix melt includes ≤ 0.25wt%Si, ≤ 0.35%wtFe, ≤ 0.05wt%Cu, ≤ 0.03wt%Mn, ≤ 0.03wt%Mg, ≤ 0.10wt%Zn, ≤ 0.10wt%Ti and > 99.60wt%Al.

According to one aspect of the present invention, wherein in step 1), prior to being added into the aluminum matrix melt, the B4C particles are preheated in an air atmosphere at 300°C-500°C for 2h-2.5h and fully dried in a vacuum drying oven.

According to one aspect of the present invention, in step 1), the aluminum matrix melt is obtained via melting the aluminum matrix under 5-10Pa vacuum and setting the aluminum matrix melt at 720°C-730°Cfor 15-20 minutes while applying mechanical stirring to the aluminum matrix melt.

According to one aspect of the present invention, in step 1), the aluminum matrix melt is subjected to standing, refining and slagging-off.

According to one aspect of the present invention, in step 1), the stirring is carried out at a temperature of 690-720°C, a stirring speed of 600-800rpm, and a mixing time of 15-30min.

According to one aspect of the present invention, in step 2), the electromagnetic field generates an electromagnetic oscillation via interaction of a constant magnetic field and a low frequency alternating magnetic field to achieve electromagnetic dispersion.

According to one aspect of the present invention, in step 2), the constant magnetic field adopts a direct current of 180A-200A, a coil turns of 80-120, a magnetic field direction of coil axis, and a magnetic field intensity of 0.1-0.4T; the low frequency alternating magnetic field adopts an alternating current of 80A-100A, a coil turns of 80-120, an alternating current frequency of 20Hz-40Hz, a magnetic field direction of coil axis, an effective magnetic field strength of 0.05-0.3T, and an oscillation time of 1.5-2min.

According to one aspect of the present invention, in step 3), the ultrasonic vibration is applied from top side, the power of the ultrasonic vibration is 240W-300W, and the vibration time of the ultrasonic vibration is 150-180s.

According to one aspect of the present invention, the twin roll continuous cast rolling uses copper twin rollers, the loading between the twin rollers is 25-30KN, the rotation speed of the twin roller is 0.9-1.2m/min, and the twin roller is cooled by water.

According to one embodiment of the present invention, a B4C/A1 neutron-absorbing material sheet is provided. The B4C/A1 neutron-absorbing material sheet is produced according to the method of the present invention.

Compared with the prior art, the method for producing B4C/A1 neutron-absorbing material sheet by continuous cast rolling of the present invention has the following advantages.
1. Twin roll continuous cast rolling can realize direct transformation from liquid to solid sheet, which can shorten the process flow, improve the processing efficiency and reduce the cost, thereby having high economic value.
2. Twin roll continuous cast rolling under coupling of ultrasonic and electromagnetic oscillation can realize quick cooling of the composite, to achieve refined grains of the solidification structure of the composite and uniform dispersion of the B4C particles without segregation.
3. Due to the ultrasonic vibration and the electromagnetic field, the B4C particles can disperse more uniformly in the matrix. The present invention is clean and free from any pollution.

Other advantages and novel features will be drawn from the following detailed description of preferred embodiments with the attached drawings. The accompanying drawings, which are incorporated in and constitute a part of this specification, illustrate embodiments of the present invention and, together with a general description of the invention given above, and the detailed description of the embodiments given below, serve to explain the principles of the invention:

### BRIEF DESCRIPTION OF THE DRAWING

Fig. 1 shows a diagram of a method for producing B4C/A1 neutron-absorbing material sheet by continuous cast rolling according to one embodiment of the present invention;
Fig. 2a shows a metallographic image (x100) of a B4C/A1 neutron-absorbing material sheet having 31% by mass of B4C particles produced according to conventional casting method under an optical microscope; and
Fig. 2b shows a metallographic image (x100) of a B4C/A1 neutron-absorbing material sheet having 31% by mass of B4C particles produced by the continuous cast rolling method of the present invention under an optical microscope.

### DETAILED DESCRIPTION OF THE INVENTION

Example embodiments of the present invention will now be described more fully hereinafter with reference to the accompanying drawings, in which some, but not all embodiments of the invention are shown. Indeed, the invention may be embodied in many different forms and should not be construed as limited to the embodiments set forth herein; rather, these embodiments are provided so that this disclosure will satisfy applicable legal requirements. Like reference numerals refer to like elements throughout.
1. Raw material selection
1) Selection of B4C particles: 325 mesh nuclear grade B4C particles produced by Mudanjiang Jingangzuan Boron Carbide Co., Ltd. are used. The particle size of the B4C particles is 0-44µm. The average grain size of the B4C particles is 18.25µm. The mass content of each chemical composition in the B4C particles is shown in the table below.

| Chemical composition | Total boron | Free boron | Total carbon | Free carbon | Fe₂O₃ | Silicon | Remaining |
|---|---|---|---|---|---|---|---|
| Mass content (%) | 79.31 | 0.23 | 19.03 | 0.58 | 0.15 | 0.05 | 0.65 |

2) Selection of the aluminum matrix: 1060 aluminum ingot is used as the aluminum matrix. The mass content of each chemical composition in the aluminum matrix is shown in the following table.

| Element | Silicon | Iron | Cooper | Manganese | Magnesium | Zinc | Titanium | Aluminum |
|---|---|---|---|---|---|---|---|---|
| Mass content (%) | ≤ 0.25 | ≤ 0.35 | ≤ 0.05 | ≤ 0.03 | ≤ 0.03 | ≤ 0.10 | ≤ 0.10 | ≥ 99.60 |

The aluminum matrix is washed in dilute hydrochloric acid, wiped via alcohol and dried for use.
2. Pretreatment of the B4C particles: 4.5kg B4C particles are preheated in air atmosphere at 300°C-500°C for 2-2.5 hours to remove impurities and moisture at the surface of the B4C particles. The preheated B4C particles are then sufficiently dried in a vacuum oven.
3. 10kg aluminum ingot is melt in a vacuum environment of 5-10Pa vacuum. The melt is set at 720°C-730°C (preferably725°C) for 15-20 minutes and subjected to mechanical agitation, so that the aluminum matrix melt has uniformly dispersed solute and temperature.
4. The aluminum matrix melt is subjected to standing, refining and slagging-off, so as to reduce air bubbles and surface oxides in the aluminum matrix melt.
5. The pretreated B4C particles are added into the aluminum matrix melt via spray method at a speed of 150g/min. While adding the B4C particles, mechanical agitation is applied to the aluminum matrix melt.
6. Composite mixing: the B4C particle-containing aluminum matrix melt is stirred at a temperature of 690-720°C (preferably700°C) with a stirring speed of 600-800rpm. The rotation speed of stirring is 750r/min at the beginning of stirring and maintained at 650r/min. The mixing time is 15-30min (preferably 20min).
7. The headbox of the continuous casting equipment of the present invention is arranged in the space between the upper and lower iron cores of the electromagnetic induction. An electromagnetic field is applied to the B4C particle-containing aluminum matrix melt passing through the headbox. The electromagnetic field generates electromagnetic oscillation via the interaction of a constant magnetic field and a low frequency alternating magnetic field to achieve electromagnetic dispersion. In the applied magnetic field as shown in Fig. 1, the constant magnetic field adopts a direct current of 180A-200A, a coil turns of 80-120, a magnetic field direction of coil axis, and a magnetic field intensity of 0.1-0.4T; the low frequency alternating magnetic field adopts an alternating current of 80A-100A, a coil turns of 80-120, an alternating current frequency of 20Hz-40Hz, a magnetic field direction of coil axis, an effective magnetic field strength of 0.05-0.3T, and an oscillation time of 1.5-2min.
8. Ultrasonic vibration is applied to the B4C particle-containing aluminum matrix melt passing through the casting nozzle. As shown in Fig. 1, the ultrasonic vibration is applied from top side, the power of the ultrasonic vibration is 240W-300W, and the vibration time is 150-180s.
9. Quick twin roll continuous cast rolling: the twin roll continuous cast rolling uses copper twin rollers. A loading between the twin rollers is 25-30KN (preferably 27KN). The rotation speed of the twin roller is 0.9-1.2m/min. The twin rollers are cooled by water. The B4C particles in the matrix can act as separating material. Therefore, there is no need to spray separating material on the rollers and the composite is free from pollution.

Is should be understood by one ordinary skilled in the art, except for the ultrasonic vibration rod and the applied magnetic field, the other components of the continuous casting equipment of the present invention are almost the same as that of the continuous casting machine in the prior art and, therefore, will not be detailed further in this application.

Compared with the prior art, the method for producing B4C/A1 neutron-absorbing material sheet by continuous cast rolling according to the present invention has the following advantages.
1. Twin roll continuous cast rolling can realize direct transformation from liquid to solid sheet, which can shorten the process flow, improve the processing efficiency and reduce the cost, thereby having high economic value.
2. Twin roll continuous cast rolling under coupling of ultrasonic and electromagnetic oscillation can realize quick cooling of the composite, to achieve refined grains of the solidification structure of the composite and uniform dispersion of the B4C particles without segregation. Fig. 2a shows a metallographic image (x100) of a B4C/A1 neutron-absorbing material having 31% by mass of B4C particles produced by conventional casting methods. Fig. 2b shows a metallographic image (x100) of a B4C/A1 neutron-absorbing material having 31% by mass of B4C particles produced by the casting method of the present invention. Via comparison of Fig. 2a and Fig. 2b, it is clearly shown that in the B4C/A1 neutron-absorbing material having 31% by mass of B4C particles produced by the conventional casting method, the B4C particles intend to aggregate and black spots intend to occur. In the B4C/A1 neutron-absorbing material having 31% by mass of B4C particles produced by the method of the present invention, the B4C particles disperse uniformly in the composite, the solidification structure is refined, and there is no noticeable defect.
3. Due to the ultrasonic vibration and the electromagnetic field, the B4C particles can disperse more uniformly in the matrix. The present invention is clean and free from any pollution.

## Claims

1. A method for producing B4C/A1 neutron-absorbing material sheet by continuous cast rolling, comprising the steps of:
1) providing B4C particles and aluminum matrix melt, adding the B4C particles into the aluminum matrix melt while stirring the composite of the B4C particles and the aluminum matrix melt;
2) applying an electromagnetic field to the B4C particle-containing aluminum matrix melt passing through a headbox;
3) applying an ultrasonic vibration to the B4C particle-containing aluminum matrix melt passing through a casting nozzle; and
4) conducing twin roll continuous cast rolling on the B4C particle-containing aluminum matrix melt from the casting nozzle to obtain B4C/A1 neutron -absorbing material sheet, and
wherein a mass content of the B4C particles in the B4C/A1 neutron-absorbing material sheet is 20-31%.

2. The method of claim 1, **characterized in that** a particle size of the B4C particles is 0-44µm.

3. The method of claim 1, **characterized in that** in step 1), the aluminum matrix melt comprises ≤ 0.25wt%Si, ≤ 0.35%wtFe, ≤ 0.05wt%Cu, ≤ 0.03wt%Mn, ≤ 0.03wt%Mg, ≤ 0.10wt%Zn, ≤ 0.10wt%Ti and ≥ 99.60wt%Al.

4. The method of claim 1, **characterized in that** in step 1), prior to being added into the aluminum matrix melt, the B4C particles are preheated in an air atmosphere at 300°C-500°Cfor 2h-2.5h and fully dried in a vacuum drying oven.

5. The method of claim 1, **characterized in that** in step 1), the aluminum matrix melt is obtained via melting the aluminum matrix under 5-10Pa vacuum and setting the aluminum matrix melt at 720°C-730°C for 15-20 minutes while applying mechanical stirring to the aluminum matrix melt.

6. The method of claim 5, **characterized in that** in step 1), the aluminum matrix melt is subjected to standing, refining and slagging-off.

7. The method of claim 1, **characterized in that** in step 1), the stirring is carried out at a temperature of 690-720°C, a stirring speed of 600-800rpm, and a stirring time of 15-30min.

8. The method of claim 1, **characterized in that** in step 2), the electromagnetic field generates an electromagnetic oscillation via interaction of a constant magnetic field and a low frequency alternating magnetic field to achieve electromagnetic dispersion.

9. The method of claim 8, **characterized in that** in step 2), the constant magnetic field adopts a direct current of 180A-200A, a coil turns of 80-120, a magnetic field direction of coil axis, and a magnetic field intensity of 0.1-0.4T; the low frequency alternating magnetic field adopts an alternating current of 80A-100A, a coil turns of 80-120, an alternating current frequency of 20Hz-40Hz, a magnetic field direction of coil axis, an effective magnetic field strength of 0.05-0.3T, and an oscillation time of 1.5-2min.

10. The method of claim 1, **characterized in that** in step 3), the ultrasonic vibration is applied from top side, a power of the ultrasonic vibration is 240W-300W, and a vibration time of the ultrasonic vibration is 150-180s.

11. The method of claim 1, **characterized in that** in step 4), the twin roll continuous cast rolling uses copper twin rollers, a loading between the twin rollers is 25-30KN, a rotation speed of the twin rollers is 0.9-1.2m/min, and the twin rollers are cooled by water.

12. A B4C/A1 neutron-absorbing material sheet produced by the method of any one of claims 1 to 11.

## Patentansprüche

1. Verfahren zur Herstellung von Neutronen-absorbierender B4C/Al-Materialfolie durch kontinuierliches Gießwalzen, umfassend die Schritte:
1) Bereitstellen von B4C-Partikeln und einer Aluminiummatrixschmelze, Zugeben der B4C-Partikel zu der Aluminiummatrixschmelze, während das Composite aus den B4C-Partikeln und der Aluminiummatrixschmelze gerührt wird,
2) Anlegen eines elektromagnetischen Feldes an die durch einen Stoffauflauf hindurchtretende B4C-Partikel enthaltende Aluminiummatrixschmelze,
3) Anlegen von Ultraschallvibration an die durch eine Gießdüse tretende B4C-Partikel enthaltende Aluminiummatrixschmelze und
4) Ausführen eines kontinuierlichen Doppelwalzen-Gießwalzens an der B4C-Partikel enthaltenden Aluminiummatrixschmelze aus der Gießdüse, um Neutronen-absorbierende B4C/Al-Materialfolie zu erhalten, und
wobei der Massengehalt der B4C-Partikel in der Neutronen-absorbieren B4C/Al-Materialfolie 20 bis 31 % beträgt.

2. Verfahren nach Anspruch 1, **dadurch gekennzeichnet, dass** die Partikelgröße der B4C-Partikel 0 bis 44 µm beträgt.

3. Verfahren nach Anspruch 1, **dadurch gekennzeichnet, dass** in Schritt 1) die Aluminiummatrixschmelze ≤ 0,25 Gew.-% Si, ≤ 0,35 Gew.-% Fe, ≤ 0,05 Gew.-% Cu, ≤ 0,03 Gew.-% Mn, ≤ 0,03 Gew.-% Mg, ≤ 0,10 Gew.-% Zn, ≤ 0,10 Gew.-% Ti und ≥ 99,60 Gew.-% Al enthält.

4. Verfahren nach Anspruch 1, **dadurch gekennzeichnet, dass** in Schritt 1) die B4C-Partikel in einer Luftatmosphäre bei 300 °C bis 500 °C 2 Stunden bis 2,5 Stunden lang vorerhitzt und in einem Vakuumtrockenofen vollständig getrocknet werden, bevor sie der Aluminiummatrixschmelze zugesetzt werden.

5. Verfahren nach Anspruch 1, **dadurch gekennzeichnet, dass** in Schritt 1) die Aluminiummatrixschmelze erhalten wird durch Schmelzen der Aluminiummatrix in einem Vakuum von 5 bis 10 Pa und Setzen der Aluminiummatrixschmelze auf 720 °C bis 730 °C für 15 bis 20 Minuten, während die Aluminiummatrixschmelze mechanischem Rühren ausgesetzt wird.

6. Verfahren nach Anspruch 5, **dadurch gekennzeichnet, dass** in Schritt 1) die Aluminiummatrixschmelze Stehen, Veredelung und Ausschlacken unterzogen wird.

7. Verfahren nach Anspruch 1, **dadurch gekennzeichnet, dass** in Schritt 1) das Rühren bei einer Temperatur von 690 bis 720 °C, bei einer Rührgeschwindigkeit von 600 bis 800 UpM und einer Rührzeit von 15 bis 30 Minuten ausgeführt wird.

8. Verfahren nach Anspruch 1, **dadurch gekennzeichnet, dass** in Schritt 2) das elektromagnetische Feld eine elektromagnetische Oszillationen erzeugt durch Interaktion eines konstanten magnetischen Feldes und eines niederfrequenten magnetischen Wechselfeldes, um eine elektromagnetische Dispersion zu erreichen.

9. Verfahren nach Anspruch 8, **dadurch gekennzeichnet, dass** in Schritt 2) das konstante magnetische Feld einen Direktstrom von 180 A bis 200 A, eine Spulenwindung von 80 bis 120, eine Magnetfeldrichtung in der Spulenachse und eine magnetische Feldstärke von 0,1 bis 0,4 T einsetzt, das niederfrequente magnetische Wechselfeld einen Wechselstrom von 80 A bis 100 A, eine Spulenwindung von 80 bis 120, eine Wechselstromfrequenz von 20 Hz bis 40 Hz, eine Magnetfeldrichtung in der Spulenachse, eine effektive Magnetfeldstärke von 0,05 bis 0,3 T und eine Oszillationszeit von 1,5 bis 2 Minuten einsetzt.

10. Verfahren nach Anspruch 1, **dadurch gekennzeichnet, dass** in Schritt 3) die Ultraschallvibration von der Oberseite angelegt wird, die Leistung der Ultraschallvibration 240 W bis 300 W beträgt und die Vibrationszeit der Ultraschallvibration 150 bis 180 Sekunden beträgt.

11. Verfahren nach Anspruch 1, **dadurch gekennzeichnet, dass** in Schritt 4) das kontinuierliche Doppelwalzen-Gießwalzen Kupfer-Doppelwalzen verwendet, eine Beaufschlagung zwischen den Doppelwalzen 25 bis 30 kN beträgt, eine Rotationsgeschwindigkeit der Doppelwalzen 0,9 bis 1,2 m/Min beträgt und die Doppelwalzen wassergekühlt werden.

12. Neutronen-absorbierende B4C/Al-Materialfolie, hergestellt durch das Verfahren nach einem der Ansprüche 1 bis 11.

## Revendications

1. Procédé de production d'une feuille de matériau absorbant neutronique B4C/Al par laminage en coulée continue, comprenant les étapes de :
1) fourniture de particules B4C et d'une fonte de matrice d'aluminium, ajout des particules B4C dans la fonte de matrice d'aluminium tout en mélangeant le composite des particules B4C et de la fonte de matrice d'aluminium ;
2) application d'un champ électromagnétique à la fonte de matrice d'aluminium contenant les particules B4C passant à travers une caisse de tête ;
3) application de vibrations ultrasonores à la fonte de matrice d'aluminium contenant les particules B4C passant à travers une buse de coulée ; et
4) réalisation d'un laminage en coulée continue à double rouleau sur la fonte de matrice d'aluminium contenant les particules B4C à partir de la buse de coulée pour obtenir une feuille de matériau absorbant neutronique B4C/Al, et
la teneur massique des particules B4C dans la feuille de matériau absorbant neutronique B4C/Al représentant 20 à 31 %.

2. Procédé selon la revendication 1, **caractérisé en ce que** la taille de particule des particules B4C représente 0 à 44 µm.

3. Procédé selon la revendication 1, **caractérisé en ce que** dans l'étape 1), la fonte de matrice d'aluminium comprend ≤ 0,25 % en poids de Si, ≤ 0,35 % en poids de Fe, ≤ 0,05 % en poids de Cu, ≤ 0,03 % en poids de Mn, ≤ 0,03 % en poids de Mg, ≤ 0,10 % en poids de Zn, ≤ 0,10 % en poids de Ti et ≥ 99,60 % en poids d'Al.

4. Procédé selon la revendication 1, **caractérisé en ce que** dans l'étape 1), avant d'être ajoutées dans la fonte de matrice d'aluminium, les particules B4C sont préchauffées dans une atmosphère d'air à 300°C à 500°C pendant 2 h à 2,5 h et complètement séchées dans un four de séchage sous vide.

5. Procédé selon la revendication 1, **caractérisé en ce que** dans l'étape 1), la fonte de matrice d'aluminium est obtenue par fusion de la matrice d'aluminium sous un vide de 5 à 10 Pa et durcissement de la fonte de matrice d'aluminium à 720°C à 730°C pendant 15 à 20 minutes tout en appliquant une agitation mécanique à la fonte de matrice d'aluminium.

6. Procédé selon la revendication 5, **caractérisé en ce que** dans l'étape 1), la fonte de matrice d'aluminium est soumise à un repos, un affinage et un décrassage.

7. Procédé selon la revendication 1, **caractérisé en ce que** dans l'étape 1), l'agitation est effectuée à une température de 690 à 720°C, une vitesse d'agitation de 600 à 800 rpm, et un temps d'agitation de 15 à 30 min.

8. Procédé selon la revendication 1, **caractérisé en ce que** dans l'étape 2), le champ électromagnétique génère des oscillations électromagnétiques par interaction d'un champ magnétique constant et d'un champ magnétique alternatif basse fréquence pour obtenir une dispersion électromagnétique.

9. Procédé selon la revendication 8, **caractérisé en ce que** dans l'étape 2), le champ magnétique constant adopte un courant continu de 180 A à 200 A, un nombre de spires de bobine de 80 à 120, la direction de champ magnétique de l'axe de bobine, et une intensité de champ magnétique de 0,1 à 0,4 T ; le champ magnétique alternatif basse fréquence adopte un courant alternatif de 80 A à 100 A, un nombre de spires de bobine de 80 à 120, une fréquence de courant alternatif de 20 Hz à 40 Hz, la direction de champ magnétique de l'axe de bobine, une intensité de champ magnétique efficace de 0,05 à 0,3 T, et un temps d'oscillation de 1,5 à 2 min.

10. Procédé selon la revendication 1, **caractérisé en ce que** dans l'étape 3), les vibrations ultrasonores sont appliquées depuis un côté supérieur, la puissance des vibrations ultrasonores vaut 240 W à 300 W, et le temps de vibration des vibrations ultrasonores représente 150 à 180 s.

11. Procédé selon la revendication 1, **caractérisé en ce que** dans l'étape 4), le laminage en coulée continue à double rouleau utilise des doubles rouleaux en cuivre, la charge entre les doubles rouleaux vaut 25 à 30 kN, la vitesse de rotation des doubles rouleaux représente 0,9 à 1,2 m/min, et les doubles rouleaux sont refroidis par de l'eau.

12. Feuille de matériau absorbant neutronique B4C/Al produite par le procédé selon l'une quelconque des revendications 1 à 11.
